

April 30, 1963

A. D. GARRISON

3,087,780

TREATMENT OF URANIUM ORE

Filed Dec. 22, 1958



## 1

3,087,780

**TREATMENT OF URANIUM ORE**  
 Allen D. Garrison, La Jolla, Calif., assignor to Texaco  
 Inc., a corporation of Delaware  
 Filed Dec. 22, 1958, Ser. No. 782,195  
 4 Claims. (Cl. 23—14.5)

This invention relates to a method of concentrating uranium values of a uranium ore. In one of its more specific aspects it is directed to an improved method of separating uranium from its ores by forming a volatilizable and sublimable uranium compound wherein said ore is contacted with a fluoride selected from the groups consisting of ammonium fluoride and ammonium bifluoride at an elevated temperature. Uranyl ammonium pentafluoride,  $(\text{UO}_2)(\text{NH}_4)_3\text{F}_5$ , is formed and is separated as a vapor from a solid ore residue. Advantageously, the ore and fluoride are contacted in the presence of an oxidizing gas, for example, air, so that any tetravalent uranium in the ore is oxidized to the hexavalent or uranyl form. The uranyl ammonium pentafluoride vapor is recovered by condensation, for example, on cooled metal pipes or walls or by contacting with cool pulverulent solids.

The uranyl ammonium pentafluoride is sublimed from the treated ore at an elevated temperature. A temperature is selected to achieve a satisfactory rate of stripping of the uranium from the ore without exceeding apparatus limitations and the temperature at which natural ingredients of the ore are sintered or melted. Since sublimation pressures are like vapor pressures and increase in like manner with increasing temperature, the uranyl ammonium pentafluoride is stripped even at temperatures below the point at which the sublimation pressure attains one atmosphere. However in order to effect rapid and complete stripping, it is preferred to contact the ore and ammonium fluoride at a temperature of at least 400° F. The upper temperature limit is wholly independent of sublimation pressure, and is determined by the melting temperature of the ore and by the limitations of the apparatus. For example, typical uranium ores may be treated at a temperature of about 1800° F. without danger of sintering and obstructing the stripping apparatus.

Uranium ores, as found in nature, usually contain large quantities of quartz and feldspars in the form of individual crystals or grains which contain little or no uranium. The uranium values appear in the cracks, crevices and grain boundaries. The quartz and feldspar are comparatively hard whereas the uranium values appear as relatively crumbly and soft interstitial films or coatings. For example, the relative hardness of some of the minerals found in uranium ores is given in the following table.

| Mineral:  | Mohs hardness |
|-----------|---------------|
| Quartz    | 7             |
| Feldspars | 6 to 6.5      |
| Uraninite | 5.5           |
| Carnotite | 2 to 4        |
| Autunite  | 2 to 2.5      |

By subjecting the ore to a scuffing or scrubbing type of grinding, the uranium values may be removed from the surface of the sand and silt particles. Desirably a grinding method is employed which selectively causes the softer interstitial material to be ground rather than the hard sand grains. Thus grinding methods which selectively crush or grind the larger grains regardless of hardness, for example, jaw crushers, ball mills, and cone grinders, are relatively ineffective for this purpose. Grinding techniques are preferred which cause the material undergoing treatment to grind itself. Autogenous grind-

## 2

ing or autoattrition methods which cause the sand grains to act as grinding agents for the softer interstitial material include for example, impingement, fluid energy grinding, jet grinding, tumbling and rolling. After grinding by an autoattrition method, the ore may be separated into coarse and fine fractions by conventional size separation techniques, the coarse fraction being of relatively lean uranium content and the fine fraction being of relatively rich uranium content.

Conventional methods of separating fine solid fractions from coarse fractions, for example, screening or centrifugal separation, may be used to concentrate the uranium values in the fine fraction. The fine fraction is readily treated by hydrometallurgical techniques for further refining. In an example of crushing and screening a uranium ore containing 0.1 percent uranium, the following fractions are produced.

| Screen size <sup>1</sup> | Weight percent uranium |
|--------------------------|------------------------|
| 60 to 100 mesh           | .02                    |
| 100 to 200 mesh          | .02                    |
| 200 to 325 mesh          | .12                    |
| 325 mesh and smaller     | .44                    |

<sup>1</sup> Screen size here and throughout this specification and claims are Tyler Standard Screen Scale.

However, separation of uranium in scuffing processes is not complete and some uranium values remain associated with the particles of sand and silt comprising the coarse fraction. Advantageously, the remaining uranium in the coarse sand fraction may be stripped therefrom by treating the coarse fraction with a substance reactive with the uranium constituents of the ore to form a sublimable compound at a temperature such that a sublimable compound is formed and condensing said sublimable compound by contact with the fine fraction to further enrich the fine fraction and recover substantially all of the uranium values of the ore. Substances reactive with the uranium constituents of ores to form sublimable compounds include halogens and halogen compounds for example, ammonium fluoride and ammonium bifluoride.

The process of this invention may be applied to the separation of uranium values from natural ores as well as from mixtures of uranium with other materials which may be produced artificially.

FIGURE 1 is a diagrammatic representation of a method of separating uranium values from an ore fraction.

FIGURE 2 is a diagrammatic representation of a method of concentrating uranium values in an ore fraction.

Although the drawings illustrate arrangements of apparatus in which the process of this invention may be practiced, it is not intended to limit the invention to the particular apparatus or materials described.

Referring to FIGURE 1, a pulverulent uranium ore in hopper 1 and ammonium fluoride from hopper 2 are passed through lines 3 and 4 respectively and combined in line 5. The ore and ammonium fluoride in admixture are introduced through line 5 into kiln 8. Kiln 8 is heated by burning air and fuel from lines 9 and 10 in burner 11. The ore and ammonium fluoride are introduced at the upper end of the kiln and are passed counter-current to the hot combustion gases from the gas burner at the lower end of the kiln. Hot flue gases containing an excess of oxygen pass over the uranium ore oxidizing any tetravalent uranium to the hexavalent or uranyl form. The uranium present in the ore reacts with the ammonium fluoride to form volatile uranyl ammonium pentafluoride which is discharged from the kiln with the gases in line 11. The hot kiln gases are passed into condenser 12 wherein the uranyl ammonium pentafluoride is solidified. Solid uranyl ammonium pentafluoride is discharged through line 15 for use or further processing not shown. Flue gas is discharged through line 16 into water scrubber 17

wherein the flue gases are contacted with water introduced through line 20 for the removal of traces of uranyl ammonium pentafluoride. Scrubbed flue gas is discharged through line 21. Water containing traces of uranyl ammonium pentafluoride is discharged through line 22 to recovery facilities not shown. Barren ore, substantially free of uranium values, is discharged from kiln 8 through line 25 for disposal or recovery of other metal values not shown.

With reference to FIGURE 2, ore in hopper 50 is passed through line 51 to attrition grinder 52. In attrition grinder 52, the ore is pulverized by impingement grinding which effects more rapid grinding of the soft components of the ore than the hard components. The ore is ground to a particle size range such that about 50 percent passes a 200 mesh sieve and 100 percent passes a 60 mesh sieve. Fine ground ore is discharged through line 53 to sieve 55. In sieve 55, the ore is separated into two fractions, a coarse fraction retained on a 200 mesh screen which is discharged through line 56 and a fine fraction passed by a 200 mesh screen which is discharged through line 57.

The coarse ore from line 56 is discharged into kiln 57 wherein it is contacted in counter-current flow with hot flue gases produced by burning fuel from line 60 and air from line 61 in burner 62. Ammonia gas from line 63 and fluorine gas from line 64 are introduced into the lower end of kiln 57 and react with the uranium values of the coarse ore to form uranyl ammonium pentafluoride. Hot flue gases containing volatile uranyl ammonium fluoride are discharged through line 70.

The fine ore fraction from sieve 55 is discharged into cooler 71. The hot flue gases containing uranyl ammonium fluoride in line 70 from kiln 57 are introduced into cooler 71 and contacted with the cold fine ore particles therein. The gas stream is cooled by contact with the fine ore and the uranyl ammonium pentafluoride condenses as a solid on the ore particles. Flue gases freed of uranyl ammonium pentafluoride are discharged through line 72. Ore, enriched in uranium values, is discharged through line 73 for further processing or use not shown.

#### Example 1

An ore containing 0.1 percent uranium is processed for the recovery of uranium values. The ore is crushed and ground to pass a 20 mesh screen in conventional crushing and grinding equipment. The 20 mesh ore fraction is then further ground in an air jet attrition grinder to pass a 60 mesh screen. The attrition mill products are then classified to separate a coarse fraction having a particle size retained on a 325 mesh screen and a fine fraction passing a 325 mesh screen. The fine fraction comprises 7.5 percent of the uranium ore and contains 0.44 percent uranium. The coarse fraction comprises 92.5 percent of the total ore and contains 0.07 percent uranium. The coarse fraction is then admixed with ammonium fluoride at a rate of 0.11 pound of ammonium fluoride per pound of coarse ore and heated in a kiln in contact with hot combustion gases containing 7.9 percent oxygen. Barren ore containing 0.01 percent uranium is discharged from the kiln. Hot flue gases from the kiln containing uranyl ammonium pentafluoride are withdrawn and condensed in the presence of the fine ore fraction to produce a fine ore concentrate having a uranium content of 1.3 weight percent.

#### Example 2

A Dakota lignite containing 0.1 percent uranium is processed for the generation carbon monoxide and hydrogen and for recovery of the uranium values. The lignite has a proximate analysis of about 30 percent moisture, 29 percent volatile matter, 29 percent fixed carbon and 12 percent ash. The lignite is reacted with steam and oxygen in relative proportions of 530 pounds of lignite (dry basis), 340 pounds of steam and 3610 standard cubic feet of substantially pure oxygen at a pressure of 205 pounds

per square inch gage and at an autogenous temperature of 2050° F. Gas of the following composition is obtained:

|                 | Mol percent, dry basis |
|-----------------|------------------------|
| Hydrogen        | 39                     |
| Carbon monoxide | 36                     |
| Carbon dioxide  | 23                     |
| Nitrogen        | 1                      |
| Methane         | 1                      |

Additionally, 106 pounds of slag comprising 0.72 weight percent uranium as  $U_3O_8$  and 14.3 weight percent carbon is withdrawn from the gas generation zone as a slurry in water. Ammonium fluoride is dissolved in the slag slurry and the slurry is then passed into a heating zone where the water is vaporized and ammonium fluoride is decomposed to ammonia gas and hydrogen fluoride gas forming a dispersion of slag particles in vapor. The slag dispersion is then passed through an attrition grinding zone and into a kiln. Air is introduced with the slag dispersion to provide an oxidizing atmosphere and further heats the slag dispersion by burning the carbon constituent of the slag. Under the high temperature oxidizing conditions of the kiln, the ammonia and hydrogen fluoride react with the uranium values of the slag forming volatile uranyl ammonium pentafluoride. The slag is separated from the vapors products which are separately cooled and solid uranyl ammonium pentafluoride is precipitated therefrom.

Obviously many modifications and variations of the invention, as hereinbefore set forth, may be made without departing from the spirit and scope thereof, and therefore only such limitations should be imposed as are indicated in the appended claims.

I claim:

1. In a process for concentrating uranium values of a uranium containing material the improvement which comprises contacting said material with a fluoride selected from the group consisting of ammonium fluoride and ammonium bifluoride in the presence of a free-oxygen containing gas at a temperature of at least 400° F., effecting formation of uranyl ammonium pentafluoride in vapor form, separating vapor comprising uranyl ammonium pentafluoride and cooling said vapor effecting formation of solid uranyl ammonium pentafluoride.

2. In a process for concentrating uranium values of a uranium containing material the improvement which comprises contacting said material with a fluoride selected from the group consisting of ammonium fluoride and ammonium bifluoride in the presence of a free-oxygen containing gas at a temperature of at least 400° F., effecting formation of uranyl ammonium pentafluoride in vapor form, separating vapor comprising uranyl ammonium pentafluoride and cooling said vapor in contact with a pulverulent solid effecting deposition of uranyl ammonium pentafluoride on said pulverulent solid.

3. In a process for concentrating uranium values of a uranium containing material the improvement which comprises contacting said material with a fluoride selected from the group consisting of ammonium fluoride and ammonium bifluoride in the presence of a free-oxygen containing gas at a temperature of at least 400° F. effecting formation of uranyl ammonium pentafluoride in vapor form, and separating vapor comprising uranyl ammonium pentafluoride from a solid residue.

4. A method of treating a uranium ore which comprises crushing said ore to pass a 60 mesh screen, classifying crushed uranium ore into a coarse fraction and a fine fraction, contacting said coarse ore fraction with a fluoride selected from the group consisting of ammonium fluoride and ammonium bifluoride in the presence of a free-oxygen containing gas at a temperature of at least 400° F. effecting formation of a sublimable uranium compound, separating said sublimable compound as a vapor from a solid ore residue, and condensing said sublimable uranium compound in contact with said fine fraction.

## References Cited in the file of this patent

## UNITED STATES PATENTS

1,070,313 Adams ----- Aug. 12, 1913  
 1,195,698 McCoy ----- Aug. 22, 1916  
 1,434,486 D'Adrian ----- Nov. 7, 1922  
 2,376,045 Gaither ----- May 15, 1945  
 2,562,024 Dunn et al. ----- July 24, 1951  
 2,580,357 McDuffie et al. ----- Dec. 25, 1951  
 2,833,617 Seaborg et al. ----- May 6, 1958

2,887,357 Seaborg ----- May 19, 1959  
 2,992,891 Sellers ----- July 18, 1961

## OTHER REFERENCES

5 Copenhofer: AEC Document NYO-5027, 7 pages, January 30, 1943, declassified February 26, 1957.  
 Katz et al.: Chemistry of Uranium, pp. 111-122 and 365 (1951), McGraw-Hill Book Co., New York.  
 Van Impe: Chem. Eng. Prog., vol. 50, No. 5, May 1954, pp. 230-234.

10